

**UNITED STATES PATENT OFFICE**

2,172,216

## PHOTOGRAPHIC DEVELOPER

Alfred Miller, Dessau, Germany, assignor, by  
mesne assignments, to Agfa Ansco Corpora-  
tion, Binghamton, N. Y., a corporation of Del-  
aware

No Drawing. Application October 27, 1938, Serial No. 237,281. In Germany October 29, 1937

1 Claim. (Cl. 95—88)

The present invention relates to photographic developers and more particularly to developers comprising additions which prevent the precipitation of lime salts from the solution.

course also on the lime content of the water used for dilution or solution. The mixtures of meta- or pyrophosphates and aliphatic nitrogenous polycarboxylic acids and their salts may be added to the concentrated developing solutions or also to the commercial dry mixtures of the development chemicals.

The following examples serve to illustrate the invention without, however, limiting the scope thereof to the specific details set forth therein. 10

### Example 1

To a developer of the following composition:

|                                                                                                                                                                   |       |      |    |
|-------------------------------------------------------------------------------------------------------------------------------------------------------------------|-------|------|----|
| 1-methylamino-4-hydroxybenzenesulfate                                                                                                                             | grams | 4    | 15 |
| Sodiumsulfite cryst.                                                                                                                                              | do    | 40   |    |
| Sodiumcarbonate                                                                                                                                                   | do    | 20   |    |
| Potassium bromide                                                                                                                                                 | gram  | 0.4  |    |
| Water                                                                                                                                                             | cc    | 1000 |    |
| there are added either in solution or to the solid mixture of chemicals 1.5 grams of sodium hexametaphosphate and 2.5 grams of trimethylamine tricarboxylic acid. |       |      |    |

*Example 2*

### Example 2

|                                       |       |      |    |
|---------------------------------------|-------|------|----|
| 1-methylamino-4-hydroxybenzenesulfate | gram  | 1    | 25 |
| Hydroquinone                          | grams | 6    |    |
| Sodiumsulfite cryst.                  | do    | 52   |    |
| Potassium carbonate                   | do    | 30   | 30 |
| Potassium bromide                     | gram  | 1    |    |
| Water                                 | cc    | 1000 |    |

### Example 3

To a developer of the following composition:

|                            |       |     |
|----------------------------|-------|-----|
| Hydroquinone               | grams | 3   |
| Sodiumsulfite sicc.        | do    | 60  |
| Sodiumcarbonate            | do    | 2   |
| Sodiumtetraborate          | do    | 4   |
| Potassium bromide          | gram  | 0.2 |
| Sodium salt of citric acid | grams | 3   |

there are added 2 grams of sodium hexameta-phosphate and 2 grams di-w.w'-methylamino-diethylamine-dicarboxylic acid. For use the developer must be dissolved in 1000 cc. of water.

I claim:

A photographic developer comprising a developing agent, an effective amount of an alkali metal salt of an acid selected from the group consisting of meta-phosphoric acid and pyrophosphoric acid and an effective amount of an aliphatic nitrogen containing polycarboxylic acid. 55

ing polycarboxylic acid.